

C. H. SMITH,

BRIQUET AND METHOD OF MAKING THE SAME.

APPLICATION FILED NOV. 15, 1916.

1,276,429.

Patented Aug. 20, 1918.



A - Coal Pile  
 B - Crusher  
 C - Hopper  
 D - Furnace  
 E - Foams (Heating)  
 F - Report in Five  
 G - Miner and Co  
 H - Discharger  
 I - Crusher  
 J - Fluxer & Mixer  
 K - Report or On  
 L - Furnace  
 M - Exhaust  
 N - Tar and Oil  
 O - Ammonia  
 P - Benzene  
 Q - Heating Co  
 S - Intermediate

Inventor

Inventor

Charles Howard Smith  
By his Attorneys  
Kidder & Morgan

# UNITED STATES PATENT OFFICE.

CHARLES HOWARD SMITH, OF SHORT HILLS, NEW JERSEY, ASSIGNOR TO INTERNATIONAL COAL PRODUCTS CORPORATION, OF RICHMOND, VIRGINIA, A CORPORATION OF VIRGINIA.

## BRIQUET AND METHOD OF MAKING THE SAME.

1,276,429.

Specification of Letters Patent.

Patented Aug. 20, 1918.

Application filed November 15, 1916. Serial No. 131,434.

*To all whom it may concern:*

Be it known that I, CHARLES HOWARD SMITH, a citizen of the United States, and a resident of Short Hills, county of Essex, and State of New Jersey, have invented new and useful Improvements in Briquets and Methods of Making the Same, of which the following is a specification.

The invention relates to briquets and methods of manufacturing the same.

One object of the invention is to produce low volatile smokeless briquets.

Another object of the invention is to form a briquet and subject it to a heating operation whereby a substantial portion of the volatile matter contained in the briquet will be distilled therefrom, leaving a strong coherent carbonized briquet which is a practically smokeless fuel.

20 I have found that when briquets are made of certain raw coals or partially carbonized coal containing approximately from eleven per cent. (11%) to seventeen per cent. (17%) volatile matter—exclusive of water which may be added in the making of the briquets—they can be heated in a manner to distil off a substantial portion of the volatile matter contained therein and that there will be left a strong coherent carbonized and substantially smokeless briquet.

35 I have also discovered that when certain soft semi-anthracite coals or partially carbonized coal, which contain less than eleven per cent (11%) volatile matter, have added thereto—in finely divided form or in liquid form—hydrocarbon volatile matter (hydrocarbon binding material), such as tar, pitch, oil or even raw coal in amount sufficient to raise the hydrocarbon matter contained in 40 the mixture to approximately from eleven per cent. (11%) to seventeen per cent. (17%)—exclusive of any water which may be added—and when the mixture is formed into a mash there can be made therefrom briquets which when subjected to a carbonizing or distilling operation lose a substantial portion of the volatile matter contained therein, leaving a strong coherent carbonized briquet which is a practically smokeless fuel.

45 50 The word "mash" as used herein is employed to designate a mass of powdered or finely divided coal or partially distilled coal having intermixed therewith water or hydrocarbon volatile matter in liquid or plastic form

whereby there results a soft mixture or 55 plastic mixture that can be readily molded into briquets.

Another object of the invention is to make carbonized smokeless briquets from high volatile coals—which as raw coals cannot, 60 because of their excess volatile content, be made into briquets that can be directly carbonized without rupture of the structure—by subjecting said high volatile coals to a preliminary distilling or carbonizing operation, by making briquets directly from the resulting residue if the volatile content in 65 said residue is of the proper proportions, or by making briquets from said resulting residue by adding thereto or mixing therewith sufficient hydrocarbon volatile matter to raise the percentage of volatile matter in the resulting mixture to the desired amount, and by subjecting the briquets thus made to a heating operation to distil therefrom 70 a substantial portion of the volatile matter contained therein, thus producing strong coherent carbonized briquets.

75 Another object of the invention is to make carbonized smokeless briquets from low volatile fuels, such as certain grades of semi-anthracite coal, or partially carbonized coal, which fuels are too low in volatile content to be formed directly into briquets, by adding such a percentage of hydrocarbon volatile matter, as an admixture or binder, as 80 will provide in the briquet sufficient volatile matter for the proper cohesion which takes place in the subsequent heating, and the subsequent heating of said briquets after their 85 formation in a manner to distil therefrom a substantial portion of the volatile matter therein, thus forming carbonized smokeless briquets.

90 95 As above indicated, one feature of the invention contemplates the making of carbonized briquets from high volatile fuel. When such fuel is employed it is prepared for formation into briquets by subjecting it to a heating operation within a substantially 100 air-tight retort so as to partially distil from the coal some of the volatile matter contained therein, chiefly the tars which come off at low temperatures and which soften and render plastic to a very large extent the 105 material under distillation. This operation may be considered an initial distillation process and it may also be referred to as the

preparing operation. During the heating, the charge within the retort is preferably constantly mixed and agitated, this being done in such a manner that all particles of 5 any particular portion of the coal mass or charge in the retort are constantly mixed or agitated whereby there will be a uniform heating and consequent distillation. In this manner the period of distillation is reduced 10 to a minimum, with a maximum recovery of by-products, and for this reason is the preferred method of initial distillation when required.

During the initial distillation the heating 15 of the coal within the retort is carried for the desired period progressively upward until a maximum temperature varying approximately from 825 degrees F. to 1200 degrees F. is reached during which heating 20 the tar vapors are largely removed. The resulting residue discharged from the retort is a dry soft partially carbonized coal (or semi-coke as some might call it) containing frome five per cent. (5%) to fourteen per 25 cent. (14%) of volatile matter. The next step of the process is the forming of this material into briquets which upon further distillation, at higher temperatures, will completely fuse or cohere in the retort into 30 strong dense blocks of the same shape as charged, and each briquet maintains this structure without disintegration or rupture upon cooling to normal temperatures.

I have found in such coals as I have tested 35 that such a cohesion does take place when the volatile matter of the briquet—exclusive of any water admixed as a temporary binder—ranges between eleven per cent. (11%) and seventeen per cent. (17%). 40 This cohesion is independent of the fact whether the briquet be composed of—

(a) certain raw coals and water;  
(b) partially carbonized coal and water;  
(c) partially carbonized coal in combination 45 with coal tar pitch, asphalt pitch, coal tar, or petroleum oils;  
(d) mixtures of coal, and either coke or partially carbonized coal, and water;  
(e) mixtures of coal, and either coke or 50 partially carbonized coal, with any of the above hydrocarbons;

(f) or a combination of any of the above with any suitable hydrocarbon;  
provided always, however, that the briqueted mixture as charged to the retort contains the proportion of volatile matter between eleven per cent. (11%) and seventeen per cent. (17%), exclusive of water.

I have found that in carbonizing briquets 60 of any of these mixtures where the percentage of volatile matter in the briquets as formed and charged to the retort is substantially less than the lower percentage mentioned (to wit, substantially less than eleven per cent. (11%)), the briquet fails to prop-

erly cohere in the furnace and disintegrates. Vice versa, I have found that where the volatile matter of the mixture substantially exceeds seventeen per cent. (17%) in the briquet as formed and charged the briquet 70 grades with increased volatile into a more or less cellular structure or a spongy coke, in which the structure of the briquet is ruptured and the briquet loses its shape and runs together into a mass while in the retort. 75

I have found that briquets made from material containing eleven per cent. (11%) to seventeen per cent. (17%) volatile matter will not run together in the retort, neither will they lose their original shape and they 80 will cohere into completely fused briquets of great strength and density. I have also found that the best results are obtained with most briquet mixtures at approximately fourteen per cent. (14%) volatile matter. 85

In forming the briquet the materials of proper volatile content as described are pulverized or rendered in a comparatively finely divided form by any suitable means, such as ordinary crushers, and thoroughly 90 and intimately mixed, after which the mixture is briqueted in any suitable manner into blocks of definite size and shape. When coal tar pitch, asphalt pitch, tar or petroleum oils form a portion of the mixture the binding can be effected in the ways well known to the art, but when coal or partially carbonized coal in a dry or non-plastic stage is used without the admixture of hydrocarbon binding material, or when a mixture 100 of partially carbonized coal and raw coal is used in a dry or non-plastic stage or condition, it is necessary to form the same into a mash, as by the admixture of sufficient water, so that this otherwise dry material 105 can be pressed or molded into the desired shape. It will be noted, however, that when partially distilled coal in a plastic condition is utilized, either to provide the whole or a part of the briquet, said plastic distilled coal 110 may provide its own binder and may be briqueted while in said plastic condition and in such case the briquetting may be accomplished without the further addition of binding material. In other words, the plastic 115 coal may be considered to provide the binding qualities necessary either when used alone or as a substantial part of the mixture.

The briquets are then charged into the second oven or retort and heated to a temperature of from 1400 degrees F. upward (preferably about 1850 degrees F.) during which heating the volatile constituents of the materials in the briquet are largely removed, a general coherence takes place and 120 the briquet is finally discharged from the oven and cooled to normal temperatures as a perfectly fused, fine grained, low volatile, free burning smokeless briquet of great 125 strength. A briquet formed of a mixture of 130

finely divided metallurgical coke and a binder when distilled in a manner so as to remove practically all of the volatile matter in the briquet—that is so as to remove all the volatile matter that is in the binder since there is practically no volatile matter in metallurgical coke—results in a briquet which is close or slow burning under ordinary drafts. A briquet made from soft, non-metallic partially distilled coal obtained at low temperatures can be redistilled at higher temperatures when mixed with pitch or other hydrocarbon binder and result in a briquet capable of ready combustion under ordinary drafts. The same is true as to briquets from which practically all of the volatile matter has been removed, that is from which all the volatile matter not only in the briquet but all the volatile matter remaining in the partially distilled coal from which the briquet has been made has been removed. The fact that the briquet last mentioned is relatively free burning is probably due to the relatively soft, non-metallic form of carbon produced by the original or initial heat treatment and which carbon is not changed or altered to a hard metallic carbon in the second or subsequent heat treatment at higher temperatures.

This feature of removing the volatile matter from the briquet and completely fusing the material composing the briquet is accomplished by my process by putting the briquet through a retort or oven which is heated to the required temperatures, as previously indicated. Manifestly, in charging the briquets to this retort or oven the briquets should be handled in such a manner that they will not be broken by rough treatment, and in such condition that they will leave the retort or oven in the shape in which they were initially formed. This retort or oven is substantially air-tight and is provided with the necessary connections to the by-product apparatus so that the products of distillation can be drawn off and recovered.

By my process I am able to take a coal having a high volatile or moisture content, or both, and by distillation reduce the percentage of volatile matter or moisture in the coal to the amount required for the manufacture of briquets which are somewhat similar in their burning characteristics to an anthracite coal. That is, I am able to concentrate a raw coal containing say thirty-six per cent. (36%) volatile matter and fifty-five per cent. (55%) fixed carbon to a briquet containing as low as two and one-half per cent. (2½%), or even lower of volatile matter and eighty-five per cent. (85%) to ninety-two per cent. (92%) of fixed carbon, according to the ash in the coal treated.

In carrying out my process I am also enabled to recover during the initial distillation of the raw coal certain by-products

contained in the coal and in addition I am also enabled to recover during the second distillation further by-products contained in the briquetted material. The residue from the initial distillation is frequently referred to as partially carbonized coal. These recoveries and the high character of the fuel make the process commercial and highly economical.

By the utilization of this process an artificial anthracite briquet, as it may be termed, viz., a briquet similar in many of its valuable properties to anthracite coal, containing two and one-half per cent. (2½%) or more or even less volatile matter can be obtained from a high volatile coal in combination with any of these binders.

The process may best be described with reference to an apparatus for carrying out the same, this apparatus and the various steps of the process being illustrated diagrammatically in the accompanying drawing forming a part of this specification. In the drawing—

Figure 1 is a diagrammatic illustration of the apparatus employed and the various steps performed. In said apparatus there is indicated one form of retort in a furnace for performing an initial heating. Figs. 2 and 3 are respectively diagrammatic longitudinal and diagrammatic transverse sectional views of another form of retort that can be employed for the initial heating.

Referring now to the drawing in detail. B represents a crusher of any suitable type adapted to crush coal received from pile A. A hopper C is provided with suitable means, such as a screw-feed or plunger, for conveying coal from the crusher to the interior of the retort F located in the furnace D. The furnace D is provided with any suitable heating means, such as flues, E, in which are located suitable gas and hot-air burners for heating the retort F.

The retort F is preferably provided with a mixer and conveyer element G comprising, for example, rotating members g having overlapping blades or paddles g'. This mixer and conveyer element G is located within the retort and is constructed and arranged so that the crushed coal which is conveyed to the interior of the retort will be uniformly and progressively heated while being mixed and conveyed through the retort. From the retort F the partially carbonized coal or resulting residue passes along a discharger and conveyer H, thence to a crusher K where it is pulverized or rendered in a finely divided form. Thence it passes to an apparatus L which comprises units for fluxing or mixing, so that the material can be brought as by the admixture of binding material to the desired percentage of volatile, and for conveying the fluxed or mixed material to a press in which the ma-

1  
terial is briqueted. The admixture previously referred to is added and mixed with the pulverized or finely divided material in the fluxing or mixing units. From the press 5 the briquets are charged or conveyed into the second retort or oven U which is located in a second furnace I. A second distillation takes place in this retort or oven and there is provided means for withdraw- 10 ing the vapors and gaseous products from the retort or oven, as will hereinafter more fully appear. The furnace I is provided with means, such as flues E, in which are located suitable gas and hot-air burners for 15 heating the retort or oven U. It will be manifest, however, that other means for heating this retort or oven may be provided, if such were desired. On completion of the 20 distillation operation the briquets are dis- charged from the oven as completely fused, coherent blocks and are allowed to at least partially cool, either before or after they have been discharged from the oven, after 25 which they may be quenched or otherwise cooled to normal temperatures.

The period the coal is left in the retort F and the amount of heat applied to the charge therein during said period is determined and controlled so that the volatile 30 content of the coal is reduced to the desired amount, approximately, for example, between five per cent. (5%) and fourteen per cent. (14%).

In order to facilitate the withdrawal of 35 the gases and vapors I provide suitable exhausting means M connected to the retorts F and U, the function of which is to maintain a balanced pressure at all times in each member to which it is connected. Suitable 40 gas outlets are also provided at both retorts for the escape and recovery of the by-products.

The mixer and conveyer element G as shown in the drawing is indicated as having 45 two shafts with overlapping paddles, but other forms of mixer and conveyer elements might be employed, for example, a single shaft  $g^2$  having paddles or conveyer members  $g^3$  thereupon. The function of this 50 mixer element G is not only to convey the material from the feed end of the retort to the discharge end, but it is also so arranged that it will continuously mix or agitate the material or charge in the retort in such a 55 manner that there will be presented a continuously changing surface or turning over of the minute granules of the material in the charge during all of the stages of heating, thus affording rapid and uniform dis- tillation.

The retort F when designed to contain as 60 a mixer element a single shaft with paddles is preferably provided with a ram or poker p arranged so as to extend—as from the discharge end of the retort—into the retort

for the purpose of overcoming any difficulty which may be incurred by the piling up or collecting of the minute material around the shaft and paddles in the retort. Such a ram or poker may at regular intervals be 70 thrust into the retort to loosen any material which may thus collect or accumulate. The method of operating the ram or poker is to thrust it into the space between the paddles, for example into a quadrant q formed by 75 the paddles when said quadrant is at the top of the retort and when the machinery is stopped. After the ram or poker has been withdrawn the machinery is operated until the next quadrant appears at the top of the 80 retort when the machinery is stopped and the ram or poker again thrust into a second quadrant. In this manner the material in each of the four quadrants may be acted 85 upon by the ram.

The gases and vapors which are given off during the heating of the coal in the retorts F and U are drawn off, as previously indicated, by the exhausting means M and they are separated by any usual or suitable condensing and distilling process into resulting by-products as, for example, tar and oil products N, ammonia O, benzene and homologues P, heating gas R, and commercial or illuminating gas S. The heating gas 90 R and the flue gases from the furnace I may be utilized for heating the retorts F and U.

In carrying out my process the coal from A is first crushed or pulverized in the crusher B. From this the crushed or pulverized coal is fed through the hopper C to the retort F in the furnace D. By means of the mixer and conveyer element G in the retort F the coal is uniformly and progressively heated throughout. The period of 10 heating and the amount of heat applied to the coal while in the retort F depend upon the character of the coal; that is, depend upon the volatile or moisture content of the coal or both of these. This also depends 11 upon the amount of volatile that it is desired to leave in the coal at the end of the initial distillation operation.

The exhausting means M draws off from 11 the retort F, during the heating operation which is performed therein, the moisture and gaseous products, the latter of which are rich in hydrocarbons that can be separated by the usual or suitable condensing and distilling processes, as desired; for example, into illuminating gas or gas for heating purposes and into tar and oil products, ammonia and other by-products, as previously indicated. The character of the heating which is performed in the second 12 oven or retort U on the briquets received from the press is dependent to a considerable extent upon the desired character of the final briquet and the amount of by-products, but a temperature of at least 1400 degrees F. is 13

recommended and 1850 degrees F. preferred on account of the yield of by-products and for the obtaining of the desired shrinkage of the briquets.

- 5 It will therefore be noted that the temperature utilized in the second oven or retort will vary according to the particular heat treatment desired. The temperature in the oven may vary from 1400 degrees F. to 2000 70 degrees F. or more, according, for example, as to whether it is desired to distil off the more highly volatile portion of the binder, or whether additional by-products not recovered at the lower temperatures, such as 10 ammonia, are desired.

A briquet produced according to this method is smokeless, durable in structure and able to withstand rough handling. It will also retain its shape during combustion. In combustion qualities it is somewhat similar to anthracite, but is consumed more readily than anthracite under the same draft. It is fine grained, dense and only slightly porous, but if the briquet be well 25 made this latter feature is not apparent to the naked eye.

As previously indicated, the purpose of the heating in the retort or oven U is to distil much of or substantially all of the 30 volatile matter contained in the briquet, and this heating operation therefore eliminates the elements, to wit, the volatile matter, which causes smoke and soot during combustion.

35 Briquets heretofore commercially made with the aid of a hydrocarbon binder have been objectionable because they have not been smokeless. According to my process I have produced a commercial briquet in 40 which a binder has been temporarily employed in the forming of the briquet, but the objectionable feature just noted has been eliminated by the performing of the second distillation operation in the retort or oven

45 U in which the volatile matter remaining in the briquet—be it the volatile matter of the binder or the volatile matter remaining in the partially carbonized coal or mixture from which the briquet was made—has been 50 in a large part removed or eliminated. In other words, I have produced a smokeless briquet made by the temporary employment of a binder which is later replaced by the coherence properties of the briquet itself.

55 According to my process there results smokeless briquets having sufficient volatile matter and sufficient porosity whereby the briquets will burn relatively free, as in an open fire without a forced draft.

60 Reference has heretofore been made to the resulting residue being a partially carbonized coal. This residue and the briquets themselves might also be described as being a concentrated fuel because a substantial 65 portion of the volatile matter contained

therein has been eliminated by the distilling or heating operation performed in the retort F and because the percentage of carbon constituent therein is materially increased as a result of the heating operation.

70 When a briquet is made in the manner above described and subjected to the second distilling operation it has been noted that a shrinkage takes place although the shape of the briquet remains unchanged; in 75 other words, the briquet finally turned out is smaller than the briquet as originally charged to the oven, it is also harder in structure, and the binder as a distinct element has disappeared. The final or resulting 80 briquet can be given a smooth surface and is comparatively clean to handle.

In carrying out such process I mix, say eighty-five per cent. (85%) of the carbon residue from the first distillation containing say ten per cent. (10%) volatile matter with say fifteen per cent. (15%) raw coal of high volatile content (say thirty-six per cent. (36%) volatile) and I thoroughly mix and pulverize the two fuels together after 90 which sufficient water is added and thoroughly mixed to form a mash and permit the mixture to be briquetted under pressure. These briquets can be made of any desired 95 shape or size and are sufficiently strong in structure to handle until they can be introduced into the second oven or retort. They are then heated to approximately 1400 degrees F. to 2000 degrees F. and discharged and quenched as previously outlined.

100 I find that in the distillation of coal the mass remains plastic until the tar vapors have been largely removed, certainly until the volatile matter has been reduced to less than 20% in the residue, and a briquet containing approximately 20% or more volatile matter and made from said residue will not retain its shape if subjected to distillation. If coal is partially distilled so that the volatile matter therein is reduced to say approxi-

105 mately between seventeen per cent. (17%) and eleven per cent. (11%), or less, then said partially distilled coal can be formed (adding hydrocarbon material if the volatile matter of the partially distilled coal is less than that desired in the briquet which is to be subsequently distilled) into briquets having approximately from eleven per cent. (11%) to seventeen per cent. (17%) volatile

110 matter, and such briquets will retain their 120 shape during a subsequent distillation performed to remove a considerable portion of the volatile matter from the briquet. I have therefore arrested the distillation at a point between these limits and molded the material into the desired shape and then continued the distillation to the desired degree. During this latter stage of the distillation the products of distillation are largely gases and vapors which will pass off without over- 130

developing the cellular structure or rupturing the briquet and beyond the shrinkage the fuel is therefore not altered in structure to any material degree. A strong free burning fuel will result from this second distillation. During the second distillation there develop some small pores resulting from the withdrawal of some of the volatile matter contained not only in the binder but also in the body material—such as the partially carbonized coal—that entered into the making of the original briquets subjected to the second distillation.

I include in this specification and consider as a part of my invention the making of smokeless briquets from (a) certain raw coal—or coals—or from partially carbonized coal—or coals—containing therein approximately from eleven per cent. (11%) to seventeen per cent. (17%) volatile matter; (b) mixtures of two or more coals—either raw or partially carbonized—containing in the mixture approximately from eleven per cent. (11%) to seventeen per cent. (17%) volatile matter; (c) mixtures of coal—or coals—either raw or partially carbonized—and coke which mixture contains approximately from eleven per cent. (11%) to seventeen per cent. (17%) volatile matter; (d) mixtures of certain raw coal—or coals—with pitch or other hydrocarbon binder or the like, mixtures of partially carbonized coal with pitch or other hydrocarbon binder or the like, mixtures of partially carbonized coal and coke with pitch or other hydrocarbon binder or the like, or mixtures of certain raw coal—or coals—and coke with pitch or other hydrocarbon binder or the like, in which mixtures the total volatile matter therein ranges from eleven per cent. (11%) to seventeen per cent. (17%) by the method which involves the forming by pressure of briquets from these fuels prior to the introduction of briquets in an oven or retort and the subsequent heating so as to distil from the briquets thus made a substantial portion of the volatile content therein, and at the same time binding the briquet so formed by their own cohesive properties.

50 The percentage of the volatile matter contained in the mixture—as the material from which the briquet is made will be referred to—may vary somewhat from the limits herein specified. This is due to the varying percentage of ash in coal and to the individual characteristics of any particular coal. The required percentage, however, can be readily determined for any particular coal and the essential characteristics of the invention will not be altered. I do not include the percentage of water utilized as a portion of the requisite percentage of volatile matter for the second distillation.

In order to give an idea as to the character 65 of briquets resulting from a particular coal

there is herein inserted, as an example, the following:

I have started with a thirty-six per cent. (36%) volatile coal having a specific gravity of 1.3 and by the initial distillation at low 70 temperatures I have reduced the volatile to approximately ten per cent. (10%) in the carbon residue which at that point had an apparent specific gravity of eight-tenths (0.8). I then crushed this material and intimately mixed with it approximately ten per cent. (10%) coal tar pitch and formed the mixture into a briquet by pressure, this briquet having approximately sixteen and one-half per cent. (16½%) volatile. 80

I then introduced this briquet into the second oven and carried the distillation up to 1850 degrees F. and allowed the briquet to slowly cool to 1400 degrees F. at which point it was removed from the oven and thoroughly cooled by quenching. After air-drying the briquet had a volatile content of two and one-half per cent. (2½%), a carbon content of approximately ninety per cent. (90%) and an apparent specific gravity of 90 1.53. I have also found by trying various other mixtures which have been outlined in the above specification that with various percentages of volatile in the briquet mixture I have been able to make briquets more or less 95 similar to those described above, all of which had an apparent specific gravity of from 1.3 or more. By this process I have succeeded in making good briquets by the use, as a binder, of kerosene, of coal tar, of certain 100 grades of petroleum oil, of asphalt pitch, and of residue from benzol stills, from all of which mixtures the results have been comparatively similar.

The expression "raw coal" used herein is 105 employed to designate coal which is the equivalent of the partially carbonized coal, which can be treated in a manner similar to the partially carbonized coal, and which can be used in my process with satisfactory re- 110 sults in place of the partially carbonized coal. These raw coals capable of such use can be readily determined by trial with any particular coal found in the locality or at hand; in other words, any particular coal 115 which it is proposed to treat.

It will be manifest that the invention herein described can be realized and performed in different ways and in different forms of apparatus without departing from 120 the spirit and scope thereof.

What I claim is:

1. The manufacture of smokeless briquets by the method which comprises heating coal and distilling therefrom at relatively low 125 temperatures a substantial portion of the volatile matter contained therein leaving a dry, soft, partially carbonized coal or residue, pulverizing said residue and mixing therewith hydrocarbon material, forming 130

the mixture into briquets and subjecting the briquets thus formed to a further distillation at higher temperatures than that of the initial distillation to distil from the briquets a substantial portion of the remaining volatile matter and cooling or quenching the briquets.

2. In the manufacture of briquets from coal or coal mixtures containing seventeen per cent. (17%) or more volatile matter the method which comprises heating coal so as to distil therefrom a limited portion of the volatile matter contained in the coal, pulverizing the residue, mixing with it binding material, forming briquets from the mixture, and heating the briquets to a temperature higher than that employed during the aforementioned distilling operation and in a manner to drive off a portion of the volatile matter contained in the briqueted binder and pulverized material.

3. In the manufacture of briquets the method which comprises taking a pulverized or finely divided coal residue of semi-coke or partially carbonized coal, mixing with said pulverized residue a hydrocarbon binder, fluxing, pressing the fluxed mixture into briquets, and subsequently heating said briquets in a manner to distil therefrom at least a part of the volatile matter contained in the briquets, the last mentioned heating being carried on in a manner to cause the elimination from the briquets of a substantial portion of ammonia derivable therefrom.

4. A briquet having ten per cent. (10%) or less in volatile matter formed by mixing a coal only partially carbonized and a hydrocarbon binder, by fluxing and pressing the mixture into briquets and by subsequently heating said briquets so as to drive off some volatile matter contained in the binder as well as in the partially carbonized coal.

5. A smokeless briquet formed of a mixture of partially carbonized coal and a binder and from which briquet a substantial portion of the volatile matter remaining in the carbonized coal and the binder has been removed by heating after briquetting.

6. The method of making briquets from high volatile coal which consists in progressively heating coal up to maximum temperature ranging from 825 degrees F. to 1200 degrees F. for a length of time which will drive off volatile matter contained therein sufficient to reduce its percentage to seventeen per cent. (17%) or less in the coal thus treated, leaving a partially distilled residue, subsequently forming a mixture of the residue and a suitable binder, and forming the resulting mixture into briquets, heating the briquets thus formed at a higher temperature than that of the first distillation and for a sufficient length of time to distil therefrom a substantial portion of the volatile

matter contained in the briquets composed of the binder and residue, and subsequently allowing said briquets to cool.

7. The method of making briquets from high volatile coal which consists in progressively heating coal up to a maximum temperature ranging from 825 degrees F. to 1200 degrees F. for a length of time which will drive off volatile matter contained therein sufficient to reduce its percentage to seventeen per cent. (17%) or less in the coal thus treated, pulverizing and forming a mixture of the residue and a suitable binder, forming the resulting mixture into briquets and heating the briquets thus formed at a higher temperature than that attained during the first heating and for a sufficient length of time to distil from the briquets a substantial portion of the volatile matter contained in the binder and residue.

8. A briquet made from partially carbonized coal and a binder by further carbonization and having a volatile content of approximately from two and a half per cent. (2½%) to ten per cent. (10%).

9. A smokeless briquet having many of the valuable properties of anthracite coal, formed by mixing partially carbonized coal and a binder and by subsequently distilling off a substantial portion of the volatile matter contained in the briquet until there is left in the briquet only approximately from two and a half per cent. (2½%) to ten per cent. (10%) volatile matter.

10. A briquet resulting from carbonizing a briquet that comprises partially carbonized coal.

11. A briquet formed by briquetting finely divided partially carbonized coal and by carbonizing after briquetting so as to remove volatile matter from the partially carbonized coal.

12. A briquet carbonized from a mixture of coal, partially carbonized, and binding material.

13. A briquet which is formed of a mixture of partially carbonized coal and a hydrocarbon binder, which briquet has been carbonized so as to eliminate a substantial portion of the volatile matter contained therein.

14. A briquet formed of a mixture of concentrated or partially distilled coal and binding material which briquet has been carbonized so as to eliminate a substantial portion of the volatile matter contained in both partially distilled coal and the binding material therein.

15. A briquet formed of a mixture of partially carbonized coal and a binder, which briquet has been carbonized as a whole so as to eliminate a substantial portion of the volatile matter in the binder and also a substantial portion of the volatile matter remaining in the partially carbonized coal, the

carbonization of the briquet being carried out in such a manner as to produce a marked shrinkage in volume and an increased apparent specific gravity of the briquet.

5 16. The process which comprises separately distilling from coal most of the tar vapors and gases which pass off at low temperatures and expand and swell the material by developing its pores, the arresting of the 10 distillation, the formation of the residue into definite pressed shapes by briquetting or the like, the resuming of the distillation, and carrying the same forward to higher temperatures than that of the first distillation to 15 further remove gases and other vapors which develop only minute cells or pores in passing from the briquets, the cells of which are substantially sealed up or closed in the contraction which takes place in the subsequent 20 cooling of the briquets.

17. A briquet produced from coal by carbonization, in which briquet the coal residue is in the form of soft non-metallic carbon that readily combines with oxygen during combustion, capable therefore of rapid combustion under draft, which briquet is free burning, tarless, burns without soot or smoke and yields a fine floury ash.

18. The manufacture of smokeless briquets by the method which comprises heating coal and distilling therefrom a portion of the volatile matter contained therein, pulverizing the resulting residue, mixing with the pulverized residue material providing 35 a hydrocarbon binder so that the total volatile matter in the resulting mixture, other than water, will approximate from eleven per cent. (11%) to seventeen per cent. (17%) in weight of the total volume 40 of the mixture, then forming the mixture into briquets and subjecting the briquets thus formed to a second operation to distil therefrom at temperatures above 1200 degrees F. a substantial portion of the volatile 45 matter contained in the briquet.

19. In the manufacture of briquets the method which comprises heating coal to temperatures of from 800 degrees F. to 1200 degrees F. so as to distill therefrom a substantial portion of the volatile matter contained therein, pulverizing the residue and mixing with the pulverized material binding material up to the point where the volatile matter in the mixture will approximate 55 from eleven per cent. (11%) to seventeen per cent. (17%) of the mixture, forming briquets from the mixture, heating the briquets to temperatures higher than said 1200 degrees F. so as to drive off a portion of the volatile matter contained in the binder and pulverized material forming the briquet in order to produce briquets of low volatile content.

20. A briquet made from a mixture of a 60 partially carbonized coal and material pro-

viding a binder, by forming under pressure the resulting mixture into briquets, and by subsequently heating said briquets so as to drive off volatile matter contained therein and so as to cause a firm union or cohesion of the particles constituting each ultimate briquet.

21. Briquets made from a mixture comprising partially carbonized coal, water and other material for providing a binder by forming, under pressure, said mixture into briquets and by subsequently heating said briquets so as to drive off volatile matter contained therein and so as to cause a firm union or cohesion of the particles constituting the ultimate briquets.

22. A briquet formed by mixing a partially carbonized coal and one or more materials providing a binder in such proportions that approximately from eleven per cent. (11%) to seventeen per cent. (17%) of the entire mixture is volatile matter, by pressing the resulting mixture into briquets, and by subsequently heating said briquets to a temperature in excess of 1200 degrees F. so as to drive off at least some of the volatile matter contained therein.

23. A smokeless briquet formed from a coal mixture or coal mash containing volatile matter approximating from eleven per cent. (11%) to seventeen per cent. (17%) of the entire mixture or mash, by pressing into briquet form and by subsequently heating the briquets thus formed at 1200 degrees F. or more so as to distil off a substantial portion of the volatile matter contained in the briquet.

24. The making of briquets by the method which comprises mixing a partially carbonized coal and hydrocarbon material providing a binder, by pressing the resulting mixture into briquets and by subsequently heating said briquets in a manner which causes a driving off of some of the volatile matter contained in the partially carbonized coal.

25. The making of briquets by the method which comprises mixing a partially carbonized coal and material providing a binder in such proportions that approximately from eleven per cent. (11%) to seventeen per cent. (17%) of the entire mixture is volatile matter, pressing the resulting mixture into briquets, and subsequently heating said briquets so as to drive off volatile matter contained in the partially carbonized coal and in the binding material.

26. The manufacture of briquets by the method which comprises forming a coal mixture or coal mash containing a high percentage of carbon, and volatile matter approximating from 11 per cent. (11%) to seventeen per cent. (17%) of the entire mixture or mash, forming said mixture or mash into briquets, and subsequently heat-

ing each briquet thus formed so as to distil off a substantial portion of the volatile matter contained in the briquet, and so as to yield a completely fused coherent briquet low in volatile matter.

27. The method which comprises mixing with coal which is either raw or partially carbonized and which has a high carbon content and low volatile content, material of high volatile content so that the volatile content of the entire mixture will approximate from eleven per cent. (11%) to seventeen per cent. (17%) thereof, forming from said mixture briquets and subsequently heating said briquets so as to distil therefrom a substantial portion of the volatile matter therein, and in a manner to leave a completely fused coherent briquet.

28. In the manufacture of briquets the method which comprises mixing with a partially carbonized coal having a high carbon content and a volatile content lower than approximately eleven per cent. (11%), a material for providing a binding material which raises the volatile content of the mixture to approximately from eleven per cent. (11%) to seventeen per cent (17%), forming briquets of the mixture and heating the briquets thus formed to sufficient temperature to distil therefrom a substantial portion of the volatile matter contained therein including a part of the volatile matter contained in the partially carbonized coal, and leaving a completely fused coherent briquet of the same general shape.

29. In the manufacture of briquets the method which comprises mixing a hydrocarbon binder with coal either raw or partially carbonized so that the volatile matter contained in the mixture will approximate from eleven per cent. (11%) to seventeen per cent (17%) adding moisture to flux the mixture, molding or pressing said mixture into briquets, and subsequently heating said briquets so as to distil therefrom a substantial portion of the volatile matter contained therein.

30. In the manufacture of briquets the method which comprises mixing together when in a pulverized condition partially carbonized coal and raw coal in such proportions that the volatile matter contained in said coals will constitute approximately from eleven per cent. (11%) to seventeen per cent. (17%) of the resulting mixture, adding moisture forming the resulting mixture into briquets and subsequently heating said briquets so as to distil therefrom a substantial portion of the volatile matter contained therein, and so as to yield a completely fused coherent briquet.

31. The manufacture of smokeless briquets from coal containing eleven per cent. (11%) to seventeen per cent (17%) volatile matter or from a mixture of coal with other mate-

rial in which mixture the volatile matter contained therein approximates from eleven per cent. (11%) to seventeen per cent. (17%) by the method which comprises forming the same when in pulverized or finely divided form into briquets by the addition of water as a temporary binder and subjecting said briquets to a carbonizing process in an inclosed retort at a temperature of from 1400 degrees F. to 2000 degrees F.

32. The manufacture of smokeless briquets from a partially carbonized coal or a mixture of partially carbonized coal and coke when in finely divided form and in which the volatile matter contained in the partially carbonized coal or mixture of partially carbonized coal and coke approximates from eleven per cent. (11%) to seventeen per cent. (17%) of the entire mass, by the method which comprises forming said partially carbonized coal or said mixture into briquets and subjecting said briquets to a carbonizing process in an inclosed retort at a temperature of from 1400 degrees F. and upward.

33. The manufacture of smokeless briquets from a mixture of coal and coke or coal partially carbonized and which mixture contains from eleven per cent. (11%) to seventeen per cent. (17%) of volatile matter, by the method which comprises forming said mixture into briquets and subjecting said briquets to a carbonizing process in an inclosed retort at a temperature to distil from the briquets a substantial portion of the volatile matter contained therein, yielding a strong coherent briquet.

34. The manufacture of smokeless briquets from a mixture of coal and coke or coal partially carbonized and which mixture contains from eleven per cent. (11%) to seventeen per cent. (17%) of volatile matter, by the method which comprises forming said mixture into briquets and subjecting said briquets to a carbonizing process in an inclosed retort at a temperature to distil off from the briquets a substantial portion of the volatile matter contained therein, and subsequently cooling said briquets by air or water.

35. The forming of briquets from coal having too high a volatile content for the direct manufacture of briquets by the method which consists in reducing said volatile content by partial carbonization in an inclosed retort so that the volatile matter contained therein will approximate from eleven per cent. (11%) to seventeen per cent. (17%) of the entire mass, then crushing the resulting residue and mixing therewith water whereby briquets can be formed and molded, forming and molding the briquets from said mixture and subsequently carbonizing in a second retort in a manner to distil from the briquets a substantial portion of the volatile

matter still remaining in the resulting residue, leaving a completely fused coherent briquet.

36. The forming of briquets from coal, coke or partially carbonized coal, or a mixture of the same in which there is too low a volatile content for the direct manufacture of smokeless fuels, by the method which comprises pulverizing said material and adding thereto sufficient hydro-carbon material to make the proportion of volatile matter contained in the resulting mixture approximate from eleven per cent. (11%) to seventeen per cent. (17%), then forming the resulting mixture into briquets by the addition of water as a temporary binder and the subsequent further carbonization of the briquets in a second retort at a temperature of approximately from 1400 degrees F. to 2000 degrees F. and subsequently cooling the briquets thus formed.

37. The forming of briquets from coal, partially carbonized coal, or a mixture of the same having too low a volatile content for the direct manufacture of smokeless briquets, by the method which consists in pulverizing the material, the adding of a sufficient quantity of hydro-carbon binder to make the proportion of volatile matter approximately from eleven per cent. (11%) to seventeen per cent. (17%), as may be required, the pressing or forming the resulting mixture into briquets, the subsequent heating of said briquets in an oven or retort at a temperature of 1400 degrees F. to 2000 degrees F. so as to distil therefrom the volatile matter contained therein so as to effect the removal and recovery of by-products given off during said distillation operation, and the quenching or cooling the resulting briquets to normal temperature.

38. The process of manufacturing low volatile briquets which process comprises initially distilling high volatile coals at sufficiently low temperatures to yield a soft, non-metallic, partially carbonized residue, briqueting this soft partially carbonized residue with the addition of such binding material as is necessary to raise the volatile matter of the briquets to approximately eleven per cent. (11%) to seventeen per cent. (17%) and subjecting the resulting briquets thus formed to a subsequent distillation at a higher temperature than that of the initial distillation in such a manner as to remove during said subsequent distillation further volatile matter from the briquets and in such a manner that there will be a substantial shrinkage in volume.

39. The process of manufacturing low volatile briquets which process comprises initially distilling high volatile coals at sufficiently low temperatures to yield a soft, non-metallic, partially carbonized residue, adding binding material to said residue and

subjecting the resulting briquets to a subsequent distillation at a higher temperature than that of the initial distillation in such a manner as to remove during said subsequent distillation further volatile matter from the briquets and in such a manner that there will be a substantial shrinkage in volume.

40. The process of manufacturing low volatile briquets which process comprises initially distilling high volatile coals at sufficiently low temperatures to yield a soft, non-metallic, partially carbonized residue, briqueting this soft partially carbonized residue after there has been added such an amount of binding material as is necessary to cause the volatile matter in the resulting briquets to approximate eleven per cent. (11%) to seventeen per cent. (17%), and subjecting said briquets to a subsequent distillation so as to remove during said subsequent distillation further volatile matter from the briquets, during which subsequent distillation a substantial shrinkage in volume takes place, the heat treatment during the subsequent distillation being such that there will not be produced hard metallic cells characteristic of coke.

41. The process of manufacturing low volatile briquets which process comprises initially distilling high volatile coals at sufficiently low temperatures to yield a soft, non-metallic, partially carbonized residue, briqueting this soft, partially carbonized residue after there has been added binding material, and subjecting said briquets to a subsequent distillation so as to remove during said subsequent distillation further volatile matter from the briquets, during which subsequent distillation a substantial shrinkage in volume takes place, the heat treatment during the subsequent distillation being such that there will not be produced hard metallic cells characteristic of coke.

42. The process of manufacturing low volatile briquets which process comprises initially distilling high volatile coals at sufficiently low temperatures to yield a non-metallic, partially carbonized residue, briqueting this partially carbonized residue after there has been added binding material comprising hydrocarbons, and subjecting said briquets to a subsequent distillation at a higher temperature so as to remove during said subsequent distillation further volatile matter from the briquets, during which subsequent distillation a substantial shrinkage in volume takes place.

43. The process of manufacturing low volatile briquets which process comprises initially distilling coals at sufficiently low temperatures to yield a soft, non-metallic, partially carbonized residue, during which initial distillation only a little, if, any shrinkage in volume that generally accom-

panies the later stage of a coking process takes place, rendering in finely divided form the partially carbonized residue, briquetting this carbonized residue either with or without the addition of binding material, if any is necessary to raise the volatile matter in the briquets to some eleven per cent. (11%) to seventeen per cent. (17%), and subjecting said briquets to a second distillation at a higher temperature to remove additional volatile matter from the briquets, the second distillation being carried out in such a manner as to cause a substantial shrinkage in volume of each briquet but so as not to produce the hard metallic cell structure characteristic of coke.

44. The process of manufacturing low volatile briquets which process comprises initially distilling coals at sufficiently low temperatures to yield a non-metallic, partially carbonized residue, during which initial distillation only a little, if any, shrinkage in volume that generally accompanies the later stage of a coke process takes place, rendering in finely divided form the partially carbonized residue, briquetting this carbonized residue, and subjecting said briquets to a second distillation at a higher temperature to remove additional volatile matter from the briquets, the second distillation being carried out in such a manner as to cause a substantial shrinkage in volume of each briquet.

45. The process of manufacturing low volatile briquets which process consists in initially distilling high volatile coal at a sufficiently low temperature to yield a soft, non-metallic, partially carbonized residue, said initial distilling operation being carried out in such a manner that little, if any, shrinkage takes place in the coal being treated, briquetting the resulting soft carbon residue so as to form briquets comprising eleven per cent. (11%) to seventeen per cent. (17%) volatile matter, and subjecting said briquets to a second distillation at a higher temperature to remove additional volatile matter from the briquets and in such a manner as to cause a substantial shrinkage in volume of the briquets.

46. The process of manufacturing low volatile briquets which process consists in initially distilling high volatile coal at a sufficiently low temperature to yield a uniform partially carbonized residue, said initial distilling operation being carried out in such a manner that little, if any, shrinkage takes place in the coal being treated, briquetting said resulting residue so as to form briquets and subjecting said briquets to a second distillation at a higher temperature to remove additional volatile matter from the briquets and in such a manner as to cause a substantial shrinkage in volume of the briquets.

47. The process of manufacturing low

volatile briquets which process consists in producing from coal by distillation a partially carbonized residue, briquetting the partially carbonized residue so as to form briquets comprising eleven per cent. (11%) to 70 seventeen per cent. (17%) volatile matter, subjecting said briquets to a second distillation at a higher temperature to remove additional volatile matter from the briquets and in such a manner to cause a substantial 75 shrinkage in volume of the briquets.

48. The making of briquets from partially carbonized coal which partially carbonized coal has previously been subjected to only a low temperature distillation 80 whereby the carbon therein would be in a relatively soft condition, by the process which comprises briquetting the partially carbonized coal and subjecting said briquets to a second distillation or carbonization 85 operation which is carried out at higher temperatures than that to which the coal was subjected prior to briquetting.

49. The making of briquets from partially carbonized coal which partially carbonized 90 coal has previously been subjected to only a low temperature distillation whereby the carbon therein is in a relatively soft condition, by the process which comprises briquetting said partially carbonized coal and subjecting said briquets to a second heating at higher temperatures than that to which the coal was subjected prior to briquetting but so as to leave the briquet sufficiently free burning to burn under ordinary 100 conditions of draft even when the volatile matter is less than two and one-half per cent. (2½%) of the total.

50. The process of treating coal consisting in first crushing said coal, then heating said coal in a manner to reduce its volatile content and to leave a soft, non-metallic, partially carbonized, relatively uniform residue, removing the gases and vapors given off by the coal during said heating, and cooling and pulverizing the residual mass.

51. The process of treating coal consisting in first crushing said coal, then heating said coal in a manner to reduce its volatile content and to leave a soft, non-metallic, relatively uniform, partially carbonized residue, removing the gases and vapors given off by the coal during said heating, cooling and pulverizing the residual mass, briquetting, and subjecting the briquets to a second heat treatment at temperatures higher than that to which the coal was subjected during the heating first referred to.

52. The process of treating coal comprising first crushing said coal, heating said crushed coal in a manner to partially remove its volatile content and in a manner to leave a soft, non-metallic, relatively uniform residue, pulverizing the residual mass, mixing therewith a suitable percentage of 125

binding material, briquetting, and carbonizing the briquets at temperatures higher than that to which the coal was first subjected.

53. The process of treating coal comprising first crushing said coal, heating said crushed coal in a manner to partially remove its volatile content and in a manner to leave a soft, non-metallic residue, pulverizing the residual mass, mixing therewith a suitable percentage of binding material, briquetting, and carbonizing the briquets at temperatures higher than that to which the coal was first subjected.

54. The process which comprises the distilling from coal of tar vapors and gases that pass off at low temperatures and expand and swell the material by developing its pores, the arresting of the distillation when the pores have been developed, the rendering of the coal residue into finely divided form, the subsequent forming of the finely divided residue, under pressure, into briquets of definite shape, and the subsequent distillation of gases and vapors from the briquets which subsequent distillation is carried forward to temperatures relatively

higher than those of the first distillation, but so as to develop only minute cells or pores within the briquets.

55. The process which comprises separately distilling from coal most of the tar vapors and gases which pass off at low temperatures and expand and swell the material by developing its pores, the arresting of the distillation, the formation of the residue into definite pressed shapes by briquetting or the like, the resuming of the distillation and the carrying of the same forward to a higher temperature than that of the first distillation to further remove gases and other vapors which develop only minute cells or pores in passing from the briquets, and allowing the briquets to cool, the last mentioned heating being carried out at temperatures sufficiently high to produce a strong coherent briquet structure.

This specification signed and witnessed this 14th day of November, A. D. 1916.

CHARLES HOWARD SMITH.

Signed in the presence of—

G. MCGRANN,

EDWIN A. PACKARD.